

## UNITED STATES PATENT OFFICE

2,271,492

## MOISTUREPROOFING COMPOSITION

William H. Bryce, Memphis, Tenn., assignor to  
Dixie Wax Paper Company, Dallas, Tex.No Drawing. Application February 23, 1939,  
Serial No. 258,102

7 Claims. (Cl. 260—736)

An object of my invention is to provide a novel coating compound for coating papers used for wrapping bread and other products.

Another object of my invention is to provide a coating compound which will render a paper for wrapping bread moisture-vapor-proof and pliable.

A further object of my invention is to provide a compound which will melt and liquefy below the boiling point of water without requiring the use of any solvent, and in which a sheet of paper may be easily dipped.

A still further object of my invention is to provide a wrapping paper for wrapping bread and other products which has a coating of a wax compound which is moisture-vapor-proof, but which coating is still not of such excessive thickness as to crack when bent and thereby render the paper opaque.

Yet another object of my invention is to provide a highly plasticized paper for wrapping candy and other products which will retain its twisted condition when used for twisting around pieces of candy and the like.

In the wrapping of bread and various other food products, and other articles, glassine paper is often used, and the present invention is particularly concerned with such glassine paper. Glassine paper is usually produced by long continued beating of pulp followed by super-calendering, and is highly transparent. Glassine pulp is highly gelatinized.

Ordinary glassine paper usually is given a thin coating of wax which is applied thereto to increase its degree of water-proofness and transparency. However, glassine paper even so treated is not entirely impervious to water vapor, and not impervious to water.

When ordinary waxed paper is used to wrap hot breads, the moisture vapor passing therethrough through its pores is likely to give it a rained-on, mottled unattractive appearance. If a very thick coating of wax is used to increase its imperviousness to water vapor and the like, such a thick layer results in the disadvantage of decreasing the transparency of the paper, leaving a tacky surface, and in hot weather or under elevated temperatures, such a wax coating will run. Further, a thick coating of wax will crack when bent or folded, leaving visible creases. On the other hand, a thin coating of wax tends to increase transparency of the paper.

I provide a glassine paper which is treated with particular substances which render it substantially moisture-vapor-proof, and at the same time highly plastic so that it may be bent without

cracking. Certain rubber derivatives are among the substances which I so employ.

Preferably, I start with a particular type of glassine paper wherein there has been incorporated during manufacture particular substances to enhance its desirable physical characteristics. A first group of substances so applied may include small percentages of a mild alkali like sodium metasilicate, or cerelose or invert or equivalent special sugar, or both. A second group of substances which may be so applied may include glycerine, glycol, magnesium chloride or zinc chloride; I use relatively more of this second group than of the first group, and ordinarily employ more of the glycerine than the other substances mentioned. A liquid containing one or more of these substances may be applied to the glassine paper sheet when near the end of its usual process of manufacture and partially dried, but still holding a considerable percentage of moisture. The mild alkali tends to increase the sheen. The cerelose improves the transparency, gloss, and moisture-proofness. The glycerine, glycol, magnesium chloride or zinc chloride are hygroscopic, and very considerably increase the pliability and the elasticity in tension, and make the paper highly plasticized.

I take glassine paper preferably of the particular type which has been described, and which has been highly plasticized, and apply thereto a thin layer of a meltable, waxy substance which not only renders the glassine paper moisture-vapor-proof, but also imparts desirable heat sealing qualities.

A preferable way to make this waxy composition is to melt some suitable wax such as a good grade of paraffin or beeswax, or the like, and dissolve therein a relatively low percentage of a suitable rubber derivative. Such waxes and the type of rubber derivatives herein described blend satisfactorily in all proportions under such a melting process without a solvent. Preferably, I use a high percentage of wax, in order to make the coated paper moisture-vapor-proof.

A rubber derivative suitable for this purpose is the substance known as "piolite" resin which is a resinous rubber addition product compound of the kind obtained by treating rubber with a compound of the type of hydrated chloro-stannic acid and precipitating the product in a finely divided state which is easily dissolved in wax; similar "piolite" resin derivatives are formed by treating rubber with a halide of an amphoteric metal. This type of rubber resin contains about 95% by weight of rubber hydrocarbon, and in the aggre-

gate is amber in color. The reaction polymerizes the rubber. Such compounds are described, for instance, in the Bruson Patent 1,848,624. It is substances of this type which I hereafter refer to as "pliolite." I use the unmilled "pliolite" resin in powdered form.

This "pliolite" resin blends with the wax in all proportions.

In one form (Formula A), of my meltable, compound for coating the glassine paper, I add a small quantity of a hydrogenated or polymerized odorless fat or oil with a melting point over 130° F., such as hydrogenated cotton-seed oil, as a lubricant to facilitate handling of the paper during manufacture. While I have in this formula indicated 10% hydrogenated cottonseed oil, this percentage may be increased or diminished within allowable limits according to lubrication conditions to be met. The hydrogenated cotton-seed oil employed should be a highly purified grade, free from objectionable odors. The commercially available product has a melting point of about 130° F. Instead of hydrogenated cottonseed oil, I may also employ hydrogenated soybean oil or hydrogenated castor oil.

I also add a small quantity of diamyl naphthalene to improve the adhesive properties of the paper under applied heat.

For certain purposes, I may also add a few percent of tricresyl phosphate ("Lindol") which acts as a plasticizer and imparts other desirable qualities.

In an improved modified form of my coating compound, (Formula B), I incorporate substantial quantities of ester gum, and also a heavy, sticky mineral oil. A suitable ester gum is rosin glyceride. A suitable oil is the product furnished by Vacuum Oil Co. under the designation P. O. 3000. This does not emulsify. I usually use about 3% mineral oil, but in some cases may use as high as 15% mineral oil. The ester gum prevents wilting or mottling of the glassine paper and makes it more moisture-vapor-proof. The ester gum also reduces the crystallinity of the waxy compound and makes it more transparent and harder. The ester gum is too brittle if applied alone without wax.

In the melt described, the ester gum will precipitate in the absence of the mineral oil which acts as a plasticizer, and hence the ester gum will be of little use, but in the presence of the plasticizer mineral oil, the ester gum will form a part of the melt. The ester gum is preferable to dammar or cumar gums, which I have also tried for this purpose. The wax with incorporated rubber resin, when melted, has still a sufficiently low viscosity so that a sheet of paper may be conveniently dipped therein. This would remain true even if relatively large percentages of rubber resin were used, but ordinarily, I use only about 5 to 10% of rubber resin.

Besides the uses of diamyl naphthalene and tricresyl phosphate as above mentioned, they also serve as plasticizers to prevent the ester gum from drying out or oxidizing out of the solution, and forming on the sides of the tank or the squeeze rolls.

While ingredients similar to some of those mentioned have been heretofore used in coating solutions for paper, they have been used in such a way as to require expensive solvents such as toluol and the like to get them into the liquid phase. I avoid the use of these expensive solvents by employing substances which when melted will all pass into the liquid phase.

One formula which I have employed with success is:

#### Formula A

|                             | Percent |
|-----------------------------|---------|
| "Pliolite" resin (powdered) | 5       |
| Hydrogenated cottonseed oil | 10      |
| Diamyl naphthalene          | 2½      |
| Paraffin wax                | 82½     |
| Total                       | 100     |

As stated, the wax may be paraffin, beeswax, or other vegetable or animal waxes of similar characteristics.

An improved formula which I have found more satisfactory in practice for general application is:

#### Formula B

|                                        | Percent |
|----------------------------------------|---------|
| "Pliolite" resin (powdered)            | 4       |
| Hydrogenated fat melting above 130° F. | 5       |
| Diamyl naphthalene                     | 1       |
| Ester gum                              | 16      |
| Heavy sticky mineral oil               | 8       |
| Paraffin wax                           | 66      |
| Total                                  | 100     |

This improved "Formula B," as stated, gives a product much less susceptible to wilting, and which is more moisture-vapor-proof.

The coating according to either "Formula A" or "Formula B" will melt at temperatures of about 175° F. to 200° F. and liquefy without the use of any solvent. The melt has a low viscosity.

A formula which I employ for low temperature or winter conditions is:

#### Formula C

|                                        | Percent |
|----------------------------------------|---------|
| "Pliolite" resin (powdered)            | 6       |
| Hydrogenated fat melting above 130° F. | 5       |
| Diamyl naphthalene                     | 1       |
| Tricresyl phosphate                    | 1       |
| Ester gum                              | 5       |
| Heavy sticky mineral oil               | 3       |
| Paraffin wax                           | 79      |
| Total                                  | 100     |

For relatively warm temperatures or summer conditions, I find the following a desirable formula:

#### Formula D

|                                        | Percent |
|----------------------------------------|---------|
| "Pliolite" resin (powdered)            | 6       |
| Hydrogenated fat melting above 130° F. | 15      |
| Diamyl naphthalene                     | 1       |
| Tricresyl phosphate                    | 1       |
| Ester gum                              | 15      |
| Heavy sticky mineral oil               | 3       |
| Paraffin wax                           | 59      |
| Total                                  | 100     |

For conditions under which the wrapper must be particularly grease-proof, the following is desirable:

#### Formula E

|                                        | Percent |
|----------------------------------------|---------|
| "Pliolite" resin (powdered)            | 4       |
| Hydrogenated fat melting above 130° F. | 40      |
| Diamyl naphthalene                     | 1       |
| Tricresyl phosphate                    | 2       |
| Ester gum                              | 40      |
| Heavy sticky mineral oil               | 3       |
| Paraffin wax                           | 10      |
| Total                                  | 100     |

In this formula, the 40% of hydrogenated cottonseed oil or other hydrogenated fat imparts grease-proofing qualities.

Under some conditions, as if a particularly good permanent seal is not important, it is possible to omit the "pliolite" resin and get fairly satisfactory results employing the following formula:

*Formula F*

|                                       | Percent    |
|---------------------------------------|------------|
| Hydrogenated fat melting above 130° F | 40         |
| Diamyl naphthalene                    | 1          |
| Tricresyl phosphate                   | 2          |
| Ester gum                             | 42         |
| Heavy sticky mineral oil              | 5          |
| Paraffin wax                          | 10         |
| <b>Total</b>                          | <b>100</b> |

This Formula F will produce a sheet which is heat-sealing, but it does not stay sealed for a length of time as will paper to which the "pliolite" formulas have been applied, but after a few days will unseal. However, I have found that sheets treated with Formula F may be made permanently heat-sealing by exuding on to one side of the sheet a concentrated rubber liquid composition, after the sheets have left the squeeze rolls after the coating of Formula F has been applied thereto and is still in melted condition, and before the sheet strikes the congealing rollers. A polishing roller smooths the composition on the sheet before it strikes the congealing rollers. A concentrated rubber composition which I have found suitable for this purpose contains 45% pliolite resin, 45% paraffin wax and 10% diamyl naphthalene. The side of the wrapping paper to which this concentrated rubber composition is applied is placed next to the food product, so that it will not come into contact with the heating elements of the automatic wrapping machine and adhere thereto.

The glassine paper may be dipped within the melt of one of these formulas at a temperature below 200° F. to form a thin coating on both sides. Also, the melt may be applied to only one side of the paper by a roller, and to the other side of the paper a coating of an ordinary wax may be applied.

For application to both sides, four pounds or more of this hot melt is applied to a ream of paper of 480 sheets of size 24 x 36 inches. Best results are obtained when applying about seven pounds of this melt to a ream of paper.

Heretofore, there have been used certain coating compositions having a very large percentage of "pliolite" and only a relatively small percentage of wax together with an expensive solvent like toluol; such compositions are necessarily expensive. On the other hand, I provide a composition with about 66% wax or more and only 4% or 5% "pliolite," and no special solvent, which is much less expensive.

The glassine paper treated with this hot melt is flexible, non-tacky, glossy, and moisture-vapor-resistant, and thermoplastic or adhesive. The treated paper also has increased tensile strength and is more resistant to the action of light and heat than the untreated paper, and is more transparent. The treated paper is tasteless, odorless, and non-toxic. The high degree of imperviousness to moisture-vapor produced makes the product which I have described, particularly suitable for wrappers for bread and other food products. After the treated paper

has been wrapped around a food product as bread, it is heat-sealed by momentarily applying to overlapping edges by a sealing hot plate, a temperature of about 175° to 200° F. which liquefies the melt including the dispersed "pliolite," and the melted "pliolite" on the two surfaces causes them to weld and seal tightly.

I have found the product which I have described to be very satisfactory in application and use, and to have decided advantages over previous compounds intended for similar purposes.

I claim:

1. A meltable wax-like composition containing from 4 to 6 percent of a powdered resinous rubber derivative, hydrogenated fat melting above 130° F., and upwards of 59 percent of a wax, said rubber derivative being the resultant of treating rubber with a halide of an amphoteric metal.

2. A meltable wax-like composition having the formula

|                                                                                        | Per cent   |
|----------------------------------------------------------------------------------------|------------|
| Resinous reaction product of rubber and an amphoteric metal halide compound (powdered) | 6          |
| Hydrogenated fat melting above 130° F                                                  | 5          |
| Diamyl naphthalene                                                                     | 1          |
| Tricresyl phosphate                                                                    | 1          |
| Ester gum                                                                              | 5          |
| Heavy sticky mineral oil                                                               | 3          |
| Paraffin wax                                                                           | 79         |
| <b>Total</b>                                                                           | <b>100</b> |

3. A meltable wax-like composition having the formula

|                                                                                        | Per cent   |
|----------------------------------------------------------------------------------------|------------|
| Resinous reaction product of rubber and an amphoteric metal halide compound (powdered) | 6          |
| Hydrogenated fat melting above 130° F                                                  | 15         |
| Diamyl naphthalene                                                                     | 1          |
| Tricresyl phosphate                                                                    | 1          |
| Ester gum                                                                              | 15         |
| Heavy sticky mineral oil                                                               | 3          |
| Paraffin wax                                                                           | 59         |
| <b>Total</b>                                                                           | <b>100</b> |

4. A meltable wax-like composition having the formula

|                                                                                        | Per cent   |
|----------------------------------------------------------------------------------------|------------|
| Resinous reaction product of rubber and an amphoteric metal halide compound (powdered) | 4          |
| Hydrogenated fat melting above 130° F                                                  | 40         |
| Diamyl naphthalene                                                                     | 1          |
| Tricresyl phosphate                                                                    | 2          |
| Ester gum                                                                              | 40         |
| Heavy sticky mineral oil                                                               | 3          |
| Paraffin wax                                                                           | 10         |
| <b>Total</b>                                                                           | <b>100</b> |

5. A wax-like composition for coating papers which may be melted and the paper dipped therein when coating the same, containing a large percentage of paraffin wax and a low percentage of an unmilled thermoplastic resinous powder prepared by treating rubber with a halide of an amphoteric metal, said thermoplastic resinous powder being added in the required proportions to increase the desired melting point of the paraffin wax and thereby increase the blocking point of the coating when passing through heat sealing means.

6. A wax-like composition for coating papers containing a large percentage of paraffin wax, an unemulsified heavy mineral oil, and a low percentage of an unmilled thermoplastic resinous powder prepared by treating rubber with a halide of an amphoteric metal.

7. A wax-like composition for coating papers

containing a large percentage of paraffin wax, a hydrogenated fat, a plasticizer, and a low percentage of an unmilled thermoplastic rubber derivative prepared by the treatment of rubber with a halide of an amphoteric metal.

WILLIAM H. BRYCE.